

May 23, 1939.

W. S. GAYLORD, JR.

2,159,693

TRANSFER

Filed Dec. 20, 1937



Inventor

William Standish Gaylord, Jr.

By Richard G Radue

Attorney

## UNITED STATES PATENT OFFICE

2,159,693

## TRANSFER

William Standish Gaylord, Jr., Summit, N. J.

Application December 20, 1937, Serial No. 180,885

11 Claims. (Cl. 41—33)

This invention relates to a new method of decoration in one or more colors for woods of all kinds, metal and metal foils, plastics of all types, painted, lacquered and varnished surfaces, cloth and textiles of all weaves and patterns, glass, and in general all kinds and types of surfaces and materials. Decorations by this method are effected by means of a transfer operating under heat and pressure. The transfer may be applied 5 by high speed machinery to any of the above mentioned surfaces and materials. The transfer operation does not depend upon the use of a liquid, as in the case of ordinary decalcomanias, nor is it dependent upon a fusible material contained in the pigmented decorative medium, nor 10 upon prior processing of the base material to be decorated. It is in these respects, among others, that it possesses novelty and special utility.

A principal object of this invention is to provide an inexpensive and practical transfer.

Another important object is the manufacture of a transfer capable of mechanical application at high production speeds. By my method, the transfer designs may be printed upon any known 25 type of printing machine, whether intaglio, typographic or planographic. The transfer may be printed either in sheets or rolls, and if printed in rolls may be transferred to the base material sought to be decorated by means of a mechanically driven heated cylinder operating at high 30 speed. If printed in sheets, the designs may be transferred to base materials by means of either a heated cylinder or a heated platen of the plate type.

Still another important object of this invention is the manufacture of a transfer from materials which are well-known, inexpensive and readily obtainable. Commercial grades of printing inks are used without modification or addition 35 of other elements. Commercial grades of paper are used as temporary carrying or backer sheets.

Another important object of this invention has been the adaptation of the process to existing 40 machinery, rather than the construction of special machinery for the manufacture of transfers.

I have reduced special processing in manufacture to a minimum and have produced a transfer 45 which can be manufactured in any ordinary printing shop. The only limitations upon the decorative work which can be done on base material by this invention are the limitations of the printing process itself.

To the best of my knowledge, no transfer has

heretofore been perfected wherein the best features of a decalcomania were combined with the best features of a heat transfer. That is to say, decalcomanias, i. e., that type of transfer which is applied by means of water soluble adhesive or its equivalent, have been free from such problems as loss of color in application, bleeding of the ink, and the like. It has been possible to print fine screen work on a wet type decalcomania paper and to reproduce multicolor work of intricate and detailed design. It has not been possible, however, to apply this type of transfer to base materials economically by mechanical means. Heat transfers, on the other hand, have permitted easy and speedy application, but with 5 definite limitations as to the scope of printing, the faithfulness of reproducing detailed designs on the base material owing to the fusible substance contained in the decorative medium used in their manufacture, and the application to non-porous surfaces, by which I mean glass, metal and the like. My invention combines the best features of each type of transfer with no limitations in printing, reproduction or application. This 10 I believe to be a new and basic improvement in 15 the field of graphic arts.

The drawing shows in perspective an elevation and section of one form of transfer together with a base material and applying means.

As illustrated in the figure of the accompanying drawing, the present invention is characterized by a temporary carrier or backer sheet of paper 1; a film 2 of thermoplastic lacquer or synthetic resin; a design layer 3 applied to the lacquer or synthetic resin and preferably composed of ordinary printing inks; a film 4 of pigmented ink, lacquer or varnish; and a film 5 of thermoplastic cement or adhesive which is fusible under 20 heat and pressure.

To effect a transfer to a base material 6, the transfer is placed with the exposed surface of the thermoplastic cement or adhesive film 5 contacting the surface of the base material. Heat and pressure are then applied to the exposed plain face of the carrier member or backer sheet 1 by means of a heated cylinder or platen 7 and a cooperating pressure member or roll 8. The heat from the cylinder or platen 7 softens the thermoplastic lacquer film 2 so as to release it from the backer sheet 1, and causes the thermoplastic cement or adhesive film 5 to fuse and grip the base material, forming a quick, strong and uniform bond. The carrier or backer sheet 1 is then stripped off, and the ink design 3 is left bonded to the base material, covered or laminated by the 25 30 35 40 45 50 55

film of thermoplastic lacquer or synthetic resin 2 which acted as a printing surface while attached to the backer sheet 1, but which has now become a tough, resilient, protective coating over the ink film or design 3, giving to the design permanence and strength which makes it resistant to friction, solvent action, and wear of other kinds.

Using a mechanically driven cylinder heated to a temperature of 200 to 250 degrees F., I have decorated 20 to 30 linear feet per minute of base material the width of the cylinder.

A platen press with a plate heated to 150 to 175 degrees F. and one to two seconds' application of pressure may be used where the base material 15 will not stand rolling pressure.

For the carrier or backer sheet of paper 1 my tests have proven that any base paper stock can be adapted, so long as it will produce a carrier which is impervious to the thermoplastic lacquer. 20 However, some paper stock is better for the purpose than others. A glassine sheet, with a base weight of from 30 to 50 pounds to the ream, is satisfactory. Standard gummed stock, such as is ordinarily sold in rolls to be used in wrapping packages, is also very satisfactory. Without 25 limiting myself to any one paper, I have found that the best results are obtained, from the point of view of strength and ease of handling, with the use of a dense kraft sheet, weighing about 30 pounds to the standard ream, and coated with the following formula:

In 400 parts by weight of water, I heat until dissolved by weight 30 parts gelatin, 1 part vegetable oil soap, 2 parts glycerine, 15 parts dextrine, 35 2 parts carbonate of soda, 2 parts boric acid, and 5 parts potash alum. After a smooth suspension is obtained and the temperature of the mixture has returned to 100 degrees F., I add to the above 5 parts egg albumin in 100 parts water.

This gives a coating material basically a colloid, the viscosity of which may be varied by more or less water, so as to control the penetration of it into the carrier or backer sheet 1, and thus control the finish of the sheet itself 45 when coated.

By varying the viscosity of the coating, I can give the backer sheet any finish I may desire, from a mat finish to a high gloss, which finish will in turn be transmitted to the film of lacquer 50 or synthetic resin 2 when a transfer is made to a base material. Four dehydrated pounds of the above solution to a standard ream, 25 inches by 38 inches and 30-lb. of paper will produce a transfer with a dull mat finish. A more viscous solution, depositing say 16 pounds of coating to the ream as above, gives a glossy finish 55 to the transferred design. The above weights, i. e., 4 and 16 pounds, designate the increase in the weight of the paper after coating and after 60 the coating has dried, and thus indicate the amount of solid material added to the ream.

This solution can be applied to the paper in a standard gumming machine. Glassine paper and the standard gummed stock mentioned above do 65 not require any additional coating and may be used as ordinarily purchased commercially. The object of this coating is to prevent penetration of the thermoplastic lacquer or synthetic resin film 2 into the carrier or backer sheet of paper, and this fact, of course, gives me an infinite 70 variety of paper stock to choose from which I may or may not treat with a special coating, as the necessity arises.

For the thermoplastic lacquer or synthetic resin 75 film 2, I have obtained good results with nitro-

cellulose and cellulose acetate base lacquers of commercial grade. Pyroxylin lacquer will also serve, as will a lacquer made of a co-polymer of vinyl chloride and vinyl acetate in acetone and amyl acetate.

A commercial synthetic resin of this nature is "Vinylite" which is manufactured by the Carbide and Carbon Chemicals Corporation. It is my practice to dissolve this resin in metho-iso-butylketone and thin it with toluol.

Improved results of a very high order have been obtained with this vinyl type lacquer. It will soften under a low heat. This property permits it to be used as a laminating agent of itself. It possesses great internal cohesion and tensile 15 strength, which properties allow it to be stripped from a backer sheet without breaking. The elasticity of the lacquer is sufficient to permit the decorated work to be shaped or even embossed without injury to the protective film on the face 20 of the transfer.

Another desirable attribute of the lacquer which has been described is that it is impervious to water, alcohol, and many of the common 25 solvents. For this reason it affords excellent protection to the transferred design.

The lacquers or synthetic resins of film 2 may be made of the proper viscosity to be applied to the carrier or backer paper 1 by means of a commercial varnishing machine, gumming machine 30 or printing machine.

The thermoplastic lacquer or synthetic resin film 2 should be clear, sheet-forming and tough. A film which will re-harden readily upon exposure to air after fusing and removal of its backer 35 sheet is ideal for many purposes to which my invention is adapted. In some cases it may be found desirable to use a rubbing and polishing lacquer where the base material to be decorated is afterwards to be refinished.

As I have already intimated, the printing or 40 decorating medium termed design 3 may be printing ink of commercial grade. A typical printing ink will be found to contain lamp-black or aniline dyes and linseed oil or mineral oils. As 45 is well known, such inks are indelible. I have used many types of commercial printing inks in the development of this invention and have found all of them to be usable without the addition of special ingredients. The general requirements 50 for the ink are those required by the type of printing being done. Inks are used as though the printing were being done on any commercial printing job. Any one skilled in the art of making printing ink can readily supply an ink possessing 55 suitable characteristics for this purpose.

The background film 4 of pigmented ink, lacquer or varnish may be applied to make the design 3 sufficiently opaque to obliterate completely 60 the base material to which it is transferred. Where a dark background is being decorated, it is sometimes necessary to increase the opacity of the design in order to obtain the desired brilliance of color. This also is accomplished by the 65 use of the film 4. On the other hand, where for example fine wood grains are being decorated by this process, it may be desirable to have the grain of the wood a part of the design. In this instance, the opacity is not desirable and the film 4 is omitted. There are no particular requirements for this film, good commercial grades of any of the media used for the purpose being easily obtainable as standard products from reputable ink and paint manufacturers.

The film of thermoplastic cement or adhesive 5 may be omitted in cases where it is not essential to the satisfactory application of the transfer. If the base material to be decorated is a 10 closely woven cloth or ground cork, for example, where the surface is porous and uniform and highly absorptive, and if a thermoplastic lacquer such as synthetic vinyl co-polymer is used as the lacquer film 2, it will be found that with the 15 application of pressure and sufficient heat to the back of the carrier paper 1, the ink design 3 and the thermoplastic vinyl resin film 2 will bond to the base material without the use of a thermoplastic cement or adhesive such as the film 5. 20 Under sufficient heat the lacquer film 2 does not merely soften to release the backer sheet paper 1, but also fuses and becomes tacky, so that the pressure will carry the softened lacquer with the 25 printed design film 3 into the fibre and/or weave of the base material, causing a firm bond thereto. 30 The thermoplastic cement or adhesive film 5 becomes tacky under heat and pressure, so as to give a quick, strong and uniform bond between the ink design and the base material to which 35 the transfer is applied. The adhesive film 5 should preferably be fusible at temperatures of 200 to 250 degrees F. It should dry rapidly and hard at room temperature and remain in such condition at shipping and handling temperatures. It should be of such viscosity as to permit 40 of its handling in a standard roller coating machine; or preferably in a printing press. It should be resistant to abrasion and chemical action. 45 I have found that lower melting resins of the phenol aldehyde group 65 parts, tri-cresyl phosphate 3 parts, tri-phenyl phosphate 6 parts, dissolved in 65 parts "Solvesso No. 1" (commercial solvent manufactured by the Standard Oil 50 Co. of New Jersey) and the whole emulsified in 30 parts water gives a very strong adhesive. Pine rosin plasticized with gum mastic in the proportion 10 rosin to 1 mastic, dissolved in "Solvesso No. 1" to the proper viscosity gives a 55 satisfactory fusible cement. By the same treatment I have adapted gutta-percha, rubber latex, and animal glue plasticized with glycerine. I have also made good thermoplastic cements 60 by using a film of overprint varnish or magnesium ground in No. 1 linseed oil dusted with 60 to 80 mesh, low-melting, powdered resins, both natural and synthetic. For this last adhesive, the varnish or magnesium film must be fresh 65 so as to hold the powder on its moist surface. Having described my invention, what I claim as new and desire to secure by Letters Patent of the United States is:

1. A transfer of the heat and pressure type 60 comprising an impervious backer sheet, a thermoplastic lacquer film on said backer sheet, a printed design on the side of the lacquer film which is opposite the backer sheet, a background 65 film of pigment covering the printed design, and

a film of thermoplastic adhesive overlying the film of pigment.

2. The combination defined in claim 1 with a backer sheet which has been rendered impervious by the application of a colloidal sizing composed of gelatin, vegetable oil soap, glycerine, dextrose, carbonate of soda, boric acid, albumin, and potash alum.

3. In a transfer of the heat and pressure type, the combination comprising an impervious backer sheet, a thermoplastic lacquer film on said backer sheet, a printed design on the side of the lacquer film opposite the backer sheet, and a background film of pigment over said printed design.

4. The combination defined in claim 3 having a backer sheet coated with a colloidal sizing of gelatin, vegetable oil soap, glycerine, dextrose, carbonate of soda, boric acid, albumin, and potash alum.

5. A transfer of the heat and pressure type which includes an impervious backer sheet, a thermoplastic lacquer film on said backer sheet, a design printed on the side of the lacquer film which is opposite the backer sheet, and a film of thermoplastic adhesive overlying said design.

6. A transfer of the heat and pressure type which includes, in combination, an impervious backer member, a thermoplastic lacquer film on said backer member, a design layer on the side of the lacquer film which is opposite the backer member, and a film of thermoplastic adhesive overlying said design layer.

7. The combination defined in claim 5 with a backer sheet which has been rendered impervious by the application of a colloidal sizing composed of gelatin, vegetable oil soap, glycerine, dextrose, carbonate of soda, boric acid, albumin, and potash alum.

8. A heat and pressure type of transfer which includes an impervious backer sheet, a thermoplastic lacquer film on said backer sheet, and a printed design on the side of the lacquer film which is opposite the backer sheet.

9. In the combination recited in claim 8, a backer sheet which has been rendered impervious by the application of a colloidal sizing composed of gelatin, vegetable oil soap, glycerine, dextrose, carbonate of soda, boric acid, albumin, and potash alum.

10. In a transfer of the heat and pressure type, the combination comprising an impervious backer sheet, a thermoplastic vinyl resin lacquer film on said backer sheet, a printed design on said film on the side opposite the backer sheet, and a film of thermoplastic adhesive overlying said design.

11. In a transfer of the heat and pressure type, the combination which includes an impervious backer sheet, a thermoplastic lacquer film comprising a co-polymer of vinyl chloride and vinyl acetate on said backer sheet, and a printed design on the film on the side opposite the backer sheet.

WILLIAM STANDISH GAYLORD, JR.